

1

2,836,152

## MEANS FOR CORRECTING HECTOGRAPHIC MASTER SHEETS

Carl Rosenblum, West Orange, N. J., assignor to Rose Ribbon & Carbon Mfg. Co., Inc., Harrison, N. J., a corporation of New York

No Drawing. Application January 19, 1955  
Serial No. 482,893

3 Claims. (Cl. 120—36)

My present invention relates generally to the art of hectographic printing, and has particular reference to the making of corrections on hectographic master sheets.

The principal object of the invention is the provision of a device for correcting such master sheets simply, economically, and without producing the messy scrapings which are characteristic of devices and methods hitherto employed.

In the "spirit" or hectographic duplicating process, a transfer sheet is used consisting of a base such as tissue paper, carrying a waxy ink coating containing spirit-soluble dye. Because such an ink coating smudges easily, and the dye discolors everything it touches, the coating is usually covered with a protective wax or other film. (A particularly desirable form of protective film, utilizing the leafing tendencies of bronze powder, is described and claimed in my Patent No. 2,671,734, issued March 9, 1954.) The desired design is transferred, by pressure from a typewriter, pencil or the like, to the under side of a master sheet, which may be of paper, plastic, aluminum foil, or the like. The preferred masters are made of clay-coated paper. When the master is completed, it carries on its under surface the design in mirror image, with the dye-carrying waxy ink coating exposed. The thin protective film of the original transfer sheet is very thin, and is largely absorbed into the clay coated surface of the master.

When errors are made in preparing masters, it is of course necessary either to remove the ink or to render it non-transferable. The latter method is practically never used, since it is generally desired to replace the mistake rather than merely to erase it. Furthermore, covering the mistake produces an uneven surface for duplicating. Hence the art has long been concerned with the problem of removing a waxy mark containing dye from a coated paper base, without unduly disturbing the base.

One conventional method involves scraping with some sharp instrument such as a knife or razor blade or glass fibered brush. This produces messy particles containing dye, and unskillful operators will destroy the coated surface of the master, so that the correction will not type in properly.

An improvement on this method involves the use of a so-called "correction pencil," which is a hard mixture of wax and clay in pencil form. It scrapes off the incorrect characters, producing debris, but the wax and clay tend to replace any coating that has been destroyed, so as to leave a surface which will accept the corrected imprint. However, this device still produces debris which tends to dirty anything with which it comes in contact.

I have discovered that it is possible selectively to remove the ink dyed wax characters from a hectographic master without the production of debris, by bringing into localized pressure contact with the selected characters a mass which under pressure is tackier than the dyed wax film, so that the ink will adhere to it, but which is insufficiently tacky to disturb or rupture the surface of the master. Pressure is applied for only a short time, and

2

then removed; on lifting the mass, it takes the ink with it. No scraping or rubbing is involved.

The pressure-sensitive mass may be formed into a pencil, but preferably it is supplied in sheet form, coated onto some carrier such as paper. The pressure sensitive mass preferably carries some dye absorbent, such as clay, bentonite, carbon black, aluminum hydrate, etc.

The selection of the ingredients of the pressure sensitive mass depends on the nature of the ink to be removed, and the strength of the paper from which it is to be lifted; the stronger the paper, the tackier the composition can be. With the general run of commercial papers and inks, certain waxes are sufficiently tacky in themselves, certain other waxes need to be tackified by additions of resin; and where the correction device is to be prepared in sheet form some waxes are sufficiently tacky, but require plasticizer to produce satisfactory adhesively coated sheets.

Beeswax, microcrystalline paraffin wax, Japan wax and most low melting petroleum pitches are sufficiently tacky to be used alone as the base of my new composition. Ordinary crystalline paraffin wax (150° F. M. P.), ceresine, Chinese insect wax, spermaceti, "Halowax," (chlorinated paraffine) and "Carbowax" (polyethylene glycol) all require some resinous tackifying addition. Typical of tack-producing addants are rosin and its derivatives, cumarone-indene and other hydrocarbon resins, rubbery materials such as polyisobutylene, and chlorinated diphenyl. Certain waxes are too hard and brittle for the contemplated purpose, and need to be plasticized. Such waxes include, for example, candellila, esparto, ouri-curi, montan, sugar cane and Utah waxes. Carnauba wax is best used with both tackifier and plasticizer. Suitable plasticizers include, for example, petrolatum, mineral oil, lard oil, sperm oil, castor oil, lanolin and low melting (120° F.) paraffin wax. Even shellac softened with Venice turpentine can be used in appropriate circumstances.

As indicated above, I prefer to employ an absorbent to help remove the ink. In general, 10 to 20% of absorbent is desirable for optimum results.

As examples of my invention, masters were prepared from transfer sheets made in accordance with my Patent No. 2,671,734, using an ink of the following composition:

|                      | Parts by weight |
|----------------------|-----------------|
| Refined Carnauba wax | 19.25           |
| Sugar cane wax       | 24.75           |
| Castor oil           | 19.25           |
| Petrolatum           | 27.5            |
| Mineral oil 100/100  | 27.5            |
| Crystal Violet       | 156.75          |

These masters could be successfully corrected with adhesive masses of the following compositions, in either film or pencil form:

|                                          | Grams |
|------------------------------------------|-------|
| "Tervan" (microcrystalline paraffin wax) | 100   |
| Candellila wax                           | 10    |
| Carbon black                             | 20    |

|                                       | Grams |
|---------------------------------------|-------|
| "Warco" microcrystalline paraffin wax | 80    |
| Sugar cane wax                        | 10    |
| China clay                            | 10    |

|                   | Grams |
|-------------------|-------|
| Carnauba wax      | 20    |
| Blown perilla oil | 20    |
| Beeswax           | 40    |
| Bentonite         | 20    |

## Example 4:

|                                |    |
|--------------------------------|----|
| Paraffin wax 135-137° F. M. P. | 10 |
| Microcrystalline paraffin wax  | 60 |
| "Alathon" (polyethylene wax)   | 10 |
| Aluminum hydrate               | 20 |

## Example 5:

|                                               |     |
|-----------------------------------------------|-----|
| "Tervan" 2536 (microcrystalline paraffin wax) | 100 |
| Carnauba wax                                  | 10  |
| Bentonite                                     | 40  |

It should be noted that these products are not pressure-sensitive adhesives in the ordinary sense; if applied to a solid surface, they will not adhere under any pressure which can be applied under ordinary circumstances. Rather, they are slightly tacky, in the sense that they will adhere lightly and immediately pull away. The important point is that they have slightly more pull than the ink, but less than the surface on which the ink is resting. The composition should in all cases be compounded in such a way that a maximum amount of tackiness is attained with due regard to the relatively small localized pressure to be employed by the user, the nature of the dye or ink to be picked up, and the quality of the paper or other material of the master sheet. The point at which fibers of the master sheet begin to be torn away is a measure of the maximum adhesive quality to be developed.

While there is no really satisfactory standard method for testing tackiness, or defining it in numerical terms, it may be noted that the wax sticks developed by Dennison Manufacturing Co. for measuring the surface bonding strength of paper (i. e., the resistance to separation of coatings or fibers) can be conveniently alluded to in describing the tackiness to be employed in the practice of the present invention. The Dennison waxes (TAPPI Standard Test #T459 m-45) are used by applying melted masses to the surface of the paper to be tested, allowing them to cool, then pulling them off. Measured in terms of these known test waxes, the ink compositions usually employed in making master sheets have a tackiness of 2A to 3A, and the new pressure-sensitive ink-removing wax compositions provided by this invention have a tackiness between 3A and 9.

When used as a coating on paper, the correction film applied may vary in thickness, preferably being from .0001 to .0020 inch in thickness.

It will thus be observed that I am successfully achieving the result desired by recourse to a phenomenon which has usually heretofore been considered a nuisance, viz., the transfer of ink from one surface to another by an act of "offsetting." For example, when carbon papers, especially "spirit" carbons, are stacked so that the inked face is in contact with the paper backing of the adjacent sheet, some of the ink will under certain conditions of pressure and temperature transfer to the adjacent sheet and make it messy. In accordance with my invention, the correction composition is so devised as to encourage this trans-

fer of dye from the sheet to be corrected to the composition that is pressed against it. Essentially, the composition is of an adhesive nature, i. e., adhesive to the ink to be lifted when a mild localized pressure is exerted; and the desired result can be attained without inclusion of an absorbent in the composition, although the addition of an absorbent ingredient is generally to be preferred. The adhesive and absorbent nature of the present composition distinguishes it from the conventional "correction pencil" whose primary ability must be its ink scraping quality, and whose friability must be such as to produce scrapings that can be readily brushed or blown away. It is just such scraping and brushing that my invention is aimed to avoid. At the same time, it should be noted that the removal of ink by the present composition is not dependent upon any softening of the waxy mass. In fact, any appreciable softening or spreading under pressure is undesirable if clean-cut accurate corrections are to result.

It will be understood that the details and proportions herein specified are in many respects set forth merely by way of example, and that changes may be made by those skilled in the art without necessarily departing from the spirit and scope of the invention as expressed in the appended claims.

Having thus described my invention what I claim as new and desire to secure by Letters Patent is:

1. A correction sheet for the removal, without rubbing or abrasion, of an unwanted spirit duplicating ink mark from a hectographic master sheet composed essentially of paper, comprising a backing sheet coated with a film of material which is only slightly tacky under moderate pressure, said material being more tacky than conventional spirit duplicating inks whereby it will remove ink from said unwanted ink mark when firmly pressed against it, but insufficiently tacky to pick fiber from the paper of which the master sheet is composed, said material comprising a major portion of wax and 10% to 20% of a filler which is an absorbent for spirit duplicating inks.

2. A correction sheet as defined in claim 1, in which the wax is predominantly microcrystalline paraffin wax.

3. A correction sheet as defined in claim 1, in which the filler is selected from the group of dye absorbents consisting of clay, bentonite, carbon black and aluminum hydrate.

## References Cited in the file of this patent

## UNITED STATES PATENTS

|           |            |               |
|-----------|------------|---------------|
| 1,399,734 | Baldwin    | Dec. 13, 1921 |
| 1,415,293 | Baldwin    | May 9, 1922   |
| 1,714,702 | Van Arsdel | May 28, 1929  |
| 1,813,675 | Moore      | July 7, 1931  |
| 1,995,685 | Perkins    | Mar. 26, 1935 |
| 2,142,761 | Quinn      | Jan. 3, 1939  |
| 2,164,035 | Jones      | June 27, 1939 |
| 2,736,911 | Larsen     | Mar. 6, 1956  |